

## UNITED STATES PATENT OFFICE

2,209,519

## PROCESS FOR PRODUCING HOLLOW CAST BLOCKS

Fritz Halbrock and Wilhelm Baumgardt, Mülheim-on-the-Ruhr, Germany, assignors to Deutsche Röhrenwerke Aktiengesellschaft, Düsseldorf, Germany, a body corporate

No Drawing. Application February 25, 1939,  
Serial No. 258,472. In Germany April 28, 1938

2 Claims. (Cl. 22—200)

It is known to produce hollow cast blocks by introducing the liquid metal into a mold; and not allowing it to solidify completely but, after a crust of the desired thickness has solidified on the 5 mold walls, upsetting the mold and thus removing the metal which is still liquid. The difficulty often arises that the head of the ingot solidifies too quickly and in an irregular shape. Even if the known covering substances are used which are 10 intended to keep the head liquid, more or less parabolically shaped boundary layers form, which make the subsequent treatment of the hollow blocks much more difficult. Furthermore, the production of predetermined wall thicknesses was 15 more or less dependent upon chance especially in the production of thick blocks. It has been found that the upper part of the block can easily be kept liquid and an approximately cylindrical shape is given to it, if a covering substance is placed on the filled mold which covering consists of a first 20 layer of a heat generating substance such as a mixture of coal, coke and aluminium, a second layer of finely ground Martin slag (slag of a steel furnace) and a third layer of chamotte powder, the layers being applied successively on the filled 25 mold in the quantitative ratio of 1:1:1. The use of heat radiating and heat insulating covering substances is known in the ordinary steel works practice. These substances are, however, 30 intended to prevent the formation of pipes. Moreover, only two layers are used. However, in the present instance the covering layers have a different purpose in view, namely to keep open the block head. Especially when the Martin slag and chamotte powder are added subsequently the 35 effect is obtained that the upper portion of the block remains liquid for a sufficiently long time,

that is until the crust has attained the desired thickness, and at the same time the hollow cast block has cylindrical shape, which is of great importance for the subsequent treatment. This applies particularly when it is desired to produce large hollow cast blocks whose wall thickness should amount to as much as  $\frac{1}{3}$  the internal diameter of the mold. The molds for still larger blocks have, for example, an internal diameter of about 2000 millimetres and a length of about 6 10 metres. The hollow blocks themselves have a wall thickness of about 400 to 500 millimetres.

We claim:

1. A process for producing heavy hollow cast steel blocks of substantially cylindrical internal shape, comprising the steps of filling a mold with molten steel, applying to the filled mold successively and in equal proportions a first layer of a heat generating composition, a second layer of finely ground Martin slag and a third layer of 15 chamotte powder, allowing the mold to cool until its steel content has solidified over a predetermined wall thickness, and then emptying the mold.

2. A process for producing heavy hollow cast steel blocks of substantially cylindrical internal shape, comprising the steps of filling a mold with molten steel, applying to the filled mold successively and in equal proportions a first layer of a mixture of coal, coke and aluminium, a second 20 layer of finely ground Martin slag and a third layer of chamotte powder, allowing the mold to cool until its steel content has solidified over a predetermined wall thickness, and then emptying the mold.

FRITZ HALBROCK.  
WILHELM BAUMGARDT.